

Jan. 15, 1935.

H. FREEMAN

1,988,416

METHOD OF PURIFYING PULP

Filed Sept. 20, 1933



Fig. 1



Fig. 2



Fig. 3.

INVENTORS:

H. FREEMAN and J. W. HUNTER

*Alex. E. MacRae*

BY

ATTORNEY.

## UNITED STATES PATENT OFFICE

1,988,416

## METHOD OF PURIFYING PULP

Horace Freeman and John Walter Hunter, Three  
Rivers, Quebec, Canada, assignors to Consol-  
idated Paper Corporation Limited, Montreal,  
Quebec, Canada

Application September 20, 1933, Serial No. 690,284  
In Canada September 21, 1932

5 Claims. (Cl. 92—20)

This invention relates to a method of treating ground wood pulp for the removal of impurities.

In the production of pulp from wood and the like there are usually present impurities which cause discolouration in the paper produced from the pulp and which have other disadvantages in the pulp. These impurities consist of particles of dirt, bark, badly discoloured fibres, pitch, rosin and the like. Moreover, long fibres and bundles of fibres may act as impurities in some classes of pulp and for the purpose of the description of the invention are to be so regarded herein.

The object of the present invention is to provide a method whereby these impurities may be readily removed from the desirable fibre leaving it free from undesirable material. The invention contemplates changing the relative buoyancy of the particles of impurities and of fibres so that they may be separated when in the form of pulp. This change in buoyancy is made possible by the difference, which has been observed, in the character of the surface of the impurities and that of the fibre. Air bubbles are thus caused selectively to adhere to the impurities and the fibre to be removed.

In the production of ground wood pulp the logs of wood are comminuted against stones and inevitably particles of knots, rosin, bark, skin, dirt and the like are formed in such a fine state of division that they may not be removed by the usual processes of screening. Owing to the usually oily or resinous character of the surface of these particles of impurities bubbles of air will cling to them. Thus, while these particles and the wood fibre are in suspension in water, the pulp is subjected to the action of air which forms bubbles about the particles of impurities. It has been found, particularly when the water is recirculated to the grinders in a more or less closed cycle, that the sugars, wood oils and the like which accumulate in the water are sufficient to constitute the necessary bubble-forming agent.

This bubble-forming and flotation step may be carried out at any stage in the treatment of the pulp but preferably after the ground wood leaves the grinders. The pulp may be caused to flow through a trough or launder with a canvas bottom through which the air is admitted to form bubbles and a top overflow trough along the sides into which the foam carrying the impurities passes while the fibre passes on to the next normal step in the process. Alternatively, the pulp may continuously flow from the grinders into a large tank, at the bottom of which air is admitted carrying the impurities to the surface from whence it is

removed while the purified fibre is continuously discharged from the tank. This may be carried out as a batch operation if desired. The air is preferably uniformly introduced near or at the bottom of the bubble-forming zone in order to afford ample opportunity for all of the particles of impurities to attach themselves to bubbles and become sufficiently buoyant to float and flow from the surface in the separating zone. The air tends to agitate the pulp but additional agitation may be employed if desired to insure liberation of all the impure particles. The foam having been removed, the pulp contains only the purified fibre which is then ready to be run into paper or used for any other purpose.

One form of apparatus for carrying out the method is disclosed in the accompanying drawing, in which:

Figure 1 is a plan view;

Figure 2 is a section on line 2—2; and

Figure 3, a section on line 3—3.

In the drawing, 1 is a trough to which the pulp is admitted by means of the inlet 2 and which has a porous bottom 3 forming an air chamber 4 supplied with an air inlet 5. Launder 4 or troughs 6 and 6' extend along the sides of the main trough 1 and are provided with outlets 7 and 7'. A dam 8 is provided adjacent the outlet end of the trough 1 to stop the forward flow of the foam and prevent its escape with the treated stock through the outlet 9 which is controlled by an adjustable weir 10.

In operation the pulp stock is admitted to the trough 1 and air under pressure is admitted to the chamber 4. In passing through the porous bottom into the stock the air forms fine bubbles which, upon rising, selectively adhere to solid portions of the stock, making the same more buoyant so that they rise to the surface with the foam and are carried off through the launders, leaving the treated stock free from the selectively removed portions. The height of the stock in the trough, the depth of the foam accumulated on the surface, and the quantity of stock which may overflow into the launders are regulated by raising or lowering the weir 10.

It will be apparent that the invention may be applied at other stages in the treatment of the pulp than those mentioned and that a great variety of means may be employed for forming the foam and effecting its removal from the pulp.

In addition to removing impurities as described the invention overcomes difficulties so frequently occasioned by the accumulation of

5

10

15

20

25

30

35

40

45

50

55

pitch giving trouble on the screens and in other parts of the equipment. Furthermore, the difficulties frequently experienced by the paper-maker due to the more or less accidental formation of foam are avoided.

It will be observed that the process is a selective one, in that it is effective in actually separating selected constituent of the pulp, leaving the remaining constituents in suspension in the fluid or water content of the pulp. In this respect it is comparable to the "flotation" process as applied to the concentration of ore. The process has wide application in the treatment of cellulose pulp and may be employed to assist screening operations or as a substitute therefor, particularly in the separation of long fibres and bundles of fibres.

We claim:

1. A method of purifying ground wood pulp which comprises passing numerous finely divided streams of air upwardly through a mass of the pulp in suspension in the water circulating through the grinder and separating the froth so formed from the pulp.
2. A method of treating ground wood pulp to remove impurities therefrom which comprises

passing numerous fine streams of air upwardly in a mass of said pulp containing water in which it was formed and removing from the surface of the pulp the froth so formed.

3. A method of purifying ground wood pulp which comprises passing fine streams of air into the pulp in substantially the condition in which it comes from the grinders to form bubbles to which impurities in the pulp adhere and removing the froth with the adhering particles.

4. A method of purifying ground wood pulp which comprises passing fine streams of air upwardly in the pulp after it leaves the grinder and before washing to form bubbles, collecting said bubbles and adhering impurities at the surface of the pulp and removing the same.

5. A method of treating ground wood pulp which comprises passing the unwashed pulp through a trough, admitting fine streams of air at the bottom of the trough to form with naturally occurring reagents in the pulp bubbles to which impurities in the pulp adhere and rise with the bubbles to the surface of the pulp and removing the bubbles and adhering impurities.

HORACE FREEMAN.

JOHN WALTER HUNTER.